

A.H. Emery  
Casting Cannon.  
No 44521. Patented Oct 4. 1864



Fig:1



Fig:4



Fig:3

Witnesses:

Charles Smith  
Edw. F. Brown

Inventor:

A.H. Emery

# UNITED STATES PATENT OFFICE.

A. H. EMERY, OF NEW YORK, N. Y.

## IMPROVEMENT IN CASTING CANNONS.

Specification forming part of Letters Patent No. 44,521, dated October 4, 1864; antedated September 24, 1864.

*To all whom it may concern:*

Be it known that J. A. H. EMERY, of the city, county, and State of New York, have invented a new and Improved Process of Founding Ordnance; and I do hereby declare that the following is a full and exact description thereof, reference being had to the accompanying drawings, and to the letters of reference marked thereon.

The nature of my invention relates to the method of casting and cooling ordnance, more especially that cooled by water from the interior, in the manufacture of which three evils have existed, which I propose to remove. These are, first, porous metal about the breech of the gun, caused by casting the gun breech down, with a chase of smaller section than the breech, the chase solidifying first, owing to its smaller section, and as the cooling progresses downward the mass of melted metal contracting draws from that solidifying in the sections above it, making these sections porous, to avoid which the chases of the guns have been made very large, and then dressed off at great expense and loss of metal, and then but partially avoiding this evil, since the chase of the gun is still left much smaller than the breech; second, the difficulty of keeping the hollow core straight and in the axis of the casting; and, third, the danger of cooling too rapidly when the hollow core has been removed by filling immediately with water.

My invention, to avoid these difficulties, consists, first, in casting the gun breech up, and continuing the casting from that part where the gun has the largest diameter when finished with a constant or increasing section up to the top thereof, which should be several inches above the end of the finished gun. Then each section will have a larger section of metal above it, so that in solidifying the metal of any one section will always solidify before that part of the casting above it solidifies, and is therefore more dense than when solidified, as heretofore, with a mass of melted metal below it, and drawing from it to make it porous, instead of giving it pressure to make it dense; second, in providing suitable ways to keep the hollow core in the axis of the casting and pass water through it, by continuing said core entirely through the casting, and subjecting it to tension after it has

been firmly secured in the axis of the mold, the tension keeping it straight; and, third, in providing ways to keep the interior of the casting rapidly cooling with water after the hollow core has been removed, until it is sufficiently cool to fill entirely with water without cooling too rapidly, by means of a pipe passing through the center of the bore, which is perforated with small holes to allow small jets of water to be forced out against the sides of the bore.

To enable others skilled in the art to make use of my invention, I will now proceed to describe it more minutely in detail.

In the drawings like figures represent like parts.

Figure 1 shows an end view of the flask and contents complete, while Fig. 2 shows a longitudinal section of the same by the cutting-plane  $z z$  in Fig. 1.

A represents the flask; B, the sand-mold containing the gun-casting C, which has been poured through the gate which is occupied by the sprue E. F is the hollow core.

The flask A is made of iron, as usual, containing the baked-sand mold B, in which the gun-casting is made with the breech up. The chase of this gun is made but little larger in the casting than it is to be when dressed, while it has to be made very much larger when the casting is made breech down, so that it may be longer in cooling, to avoid porosity of the part below it, which still has a larger section, so that it only partially counteracts this evil, while it has to be dressed off at great expense.

The difficulty of introducing water to the hollow core, as heretofore used when cast with the breech up, has prevented their use entirely, as the work would all have to be done at the bottom of a highly-heated pit in which the casting is being made. I pass these hollow cores entirely through the casting, so I can work at them from the top, where I can readily get at them, even when the pit is heated.

Instead of rounding off the casting at the breech, as heretofore, I continue it the size of the largest part, or increasing up to the top of the casting, which is carried sufficiently above the end of the finished gun to give the required density at the end of the finished gun. It will be seen that the casting has an increasing section from the muzzle at the bottom up to the

top, so that each section solidifies with a head of melted metal above it equal to its distance from the top of the gun-casting, and is therefore very dense and free from pores.

In casting cannons which have small bores the difficulties of keeping the cores straight and in the axis of the casting have wholly prevented their being water-cooled from the interior. By passing the hollow core entirely through the casting, and then keeping it under tension while it is firmly secured in the axis of the mold while casting, it is kept straight and in its proper position while water is circulating through it.

In the drawings, D shows a cross-piece attached to the flask, through which the hollow core F passes, and I shows a sleeve through which it passes at the bottom, these two pieces D and I securing the ends of the hollow core F in the axis of the mold. It is kept straight by means of the screws K and H and rubber spring G, by which it is kept under a strain of tension.

After the metal has all solidified the hollow core F is removed, the sleeve I taken out, and a ring of soft clay placed on the upper end of it, and the sleeve I is then screwed back, when the clay ring will keep the water from getting between the sleeve I and casting C into the sand mold B when the gun is filled with water, but does not prevent the water from passing

through the bore and sleeve. After the sleeve I is put in its place the pipe L (shown in Figs. 3 and 4) is put in the bore of the gun, and a stream of water circulated through it while it is slowly rotated. This pipe is perforated with small holes, which allow fine streams of water to be forced out against the sides of the bore, thus cooling it rapidly, but not too fast. When the temperature of the interior of the casting that is along the surface of the bore is reduced to about boiling-heat of water, the bore may be entirely filled with water, which must circulate rapidly to prevent a rapid formation of steam, this circulation being kept up until the casting is nearly or quite cold.

What I here claim, and desire to secure by Letters Patent, is—

1. Casting cannons with the breech uppermost, as and for the purpose described, and with the hollow-core bar or mandrel passing through and projecting beyond both ends of the casting.
2. In the casting of cannons, applying to the hollow-core bar a tensile strain, substantially in the manner and for the purpose described.
3. The use of the water-pipe L, substantially as and for the purpose set forth.

A. H. EMERY.

Witnesses:

CHARLES SMITH,  
EDM. F. BROWN.